

## UNITED STATES PATENT OFFICE

1,951,207

DISTILLATE PETROLEUM PRODUCT AND  
METHOD OF TREATING SAME

James B. Rather, Brooklyn, Orland M. Reiff,  
Jackson Heights, and Leslie C. Beard, Jr.,  
Brooklyn, N. Y., assignors to Socony-Vacuum  
Corporation, New York, N. Y., a corporation of  
New York

No Drawing. Application April 23, 1929,  
Serial No. 357,603

7 Claims. (Cl. 44—9)

This invention relates to distillate petroleum products, more particularly gasoline and kerosene, and to a method of and means for imparting a stability thereto with respect to color, 5 gum formation and odor and for removing any objectionable color developed therein during storage.

This application is a continuation in-part of our co-pending applications Serial No. 315,914 filed October 29, 1928, Serial No. 151,005, filed November 26, 1926 and Serial No. 165,546 filed February 3, 1927.

It is well known that during storage, the lighter refined petroleum distillates, notably gasoline and kerosene, frequently become discolored and develop a quantity of gummy material and an objectionable odor, as a result, it is generally believed, of atmospheric oxidation. And it is known that cracked gasoline will generally accumulate a gummy material during comparatively short periods of storage, particularly in the glass bowls of visible service pumps.

This discoloration and odor developed in gasoline and kerosene are objectionable to consumers and distributors of these products and the presence of gummy material in gasoline causes such undesirable effects, when used in internal combustion engines, as sticking of the valve stems and excessive carbon formation.

In accordance with this invention, however, the development of these undesirable characteristics in distillate petroleum products may be readily prevented or materially delayed and any discoloration may be effectually removed and 35 without appreciably increasing the cost of production thereof.

One of the objects, therefore, of this invention, is to provide a method of and means for preventing or materially delaying the development of discoloration, objectionable odor and the formation of gummy material in distillate petroleum products.

Another object of the invention is to provide a method of and means for removing objectionable color developed in distillate petroleum products and for preventing initial and recurrent discoloration thereof.

Another object of the invention is to provide agents or compounds effective both as decolorizers and color stabilizers of distillate petroleum products and also effective to prevent or materially delay the formation of gum and objectionable odor therein.

Another object of the invention is to provide 55 a method and means of the character referred

to that will not appreciably increase the cost of production of distillate petroleum products.

Other objects of the invention will be apparent from the following description.

We have discovered that certain of the hydroxy compounds, such as the hydroxy benzenes and particularly the trihydroxy benzenes are effective as decolorizers and stabilizers with respect to color, gum formation and odor of distillate petroleum products of A. P. I. gravity 60 higher than 37°. Of the trihydroxy benzenes, pyrogallol is preferably employed because, in addition to its effectiveness in decolorization and color and odor stabilization, it is probably the most effective of the trihydroxy benzenes in preventing or delaying the formation of gum in petroleum distillates.

The method employed preferably comprises the thorough mixing of a relatively minute amount of the agent or compound, such as pyrogallol, 75 with the distillate to be treated, although it will be understood that the distillate may be percolated through a mass of the agent or compound, if desired. Preferably, however, the pyrogallol is first dissolved in a suitable solvent which is 80 miscible with the distillate, such as acetone or an aliphatic alcohol, as isopropyl, ethyl or butyl alcohol, in the proportion of approximately one part of pyrogallol to ten parts of the solvent. The resulting solution is then added to the distillate to be treated in the desired proportion. By this method the pyrogallol is distributed 85 throughout and dissolved in the distillate more readily than if it were added directly thereto.

It has been found that as little as one part 90 by weight of pyrogallol to approximately 75,000 parts of distillate is an effective proportion for decolorizing and for preventing the development of objectionable color, odor and the formation of gum. Somewhat larger proportions 95 may be used, if desired, but the absorption of too large a quantity of the agent or compound may result in discoloration due to the compound imparting its own color to the distillate. In most instances, however, the distillate will absorb only a limited amount of the compound and if the process is carried on at ordinary temperatures, there will be no danger of the absorption of an objectionable or quality impairing quantity of the same.

As an example of the practice of this invention, a 10% solution of the compound, as pyrogallol, in isopropyl alcohol may be prepared, or, five pounds of pyrogallol may be dissolved in five gallons of isopropyl alcohol. The pyro-

gallol solution is then added gradually to the distillate to be treated and preferably in such quantities that the ratio of the amount of pyrogallol to the distillate will be approximately one 5 part by weight of pyrogallol to 75,000 parts of distillate. After the pyrogallol and the distillate have been thoroughly mixed, the resulting solution is conducted into a clean, dry tank, and allowed to stand until the reaction of the 10 pyrogallol with the distillate is complete. At ordinary temperatures, this usually requires about 24 hours, but at higher temperatures, the time required may be somewhat less. During this treatment the distillate should preferable 15 be kept out of contact with water otherwise the agent or compound may be dissolved in the water and possibly result in the return of some degree of discoloration.

Tests have shown that a distillate petroleum 20 product having an initial color of -9 Saybolt Chromometer, when treated with as little as one part of pyrogallol to 75,000 parts of the distillate and allowed to stand for only two hours, had a color of +18 Saybolt, thus showing an improvement in color of 27 points Saybolt.

The gum forming tendency of distillate petroleum products, such as gasoline, for example, may be effectually measured by the evaporation 30 of the gasoline in a copper cup according to the United States Bureau of Mines Method 530.1, Technical Paper 323B. Tests in accordance with this method have shown that with commercial samples of unrefined gasoline distillate, the amount of gum formed by the evaporation of the gasoline in a copper cup prior to treatment with pyrogallol amounted to 288 milligrams, whereas after treatment with as little 35 as one part of pyrogallol dissolved in 75,000 parts of the gasoline, only 7 milligrams were formed.

The foregoing treatment has been found most satisfactory and effective in the decolorization and stabilization of distillate petroleum products of A. P. I. gravity higher than 37° with respect to color, gum formation and odor, and is particularly advantageous because it does not appreciably increase the cost of production or the handling charges thereof.

50 While we have thus specifically described our invention, various modifications thereof may suggest themselves to those skilled in the art, and it is therefore our intention that the invention be limited only by the scope of the appended claims.

Having thus described our invention, what we claim and desire to secure by Letters Patent is:

1. A low boiling normally light colored distillate petroleum product of the class of gasoline or kerosene which normally tends to become discolored during storage, having added 60

thereto a polyhydroxy-benzene effective to, and in quantity sufficient to, substantially retard spontaneous discoloration of the product.

2. The method of stabilizing the characteristics of a low boiling normally light colored distillate petroleum product of the class of gasoline or kerosene that normally tends to become discolored during storage, which comprises adding thereto prior to substantial spontaneous discoloration a small quantity of a polyhydroxy-benzene sufficient substantially to retard self-generated discoloration of the product.

3. A low boiling normally light colored distillate petroleum product of the class of gasoline or kerosene which normally tends to become discolored during storage, having added thereto a trihydroxy-benzene in quantity sufficient substantially to retard spontaneous discoloration of the product.

4. The method of stabilizing the characteristics of a low boiling normally light colored distillate petroleum product of the class of gasoline or kerosene that normally tends to become discolored during storage, which comprises adding thereto prior to substantial spontaneous discoloration a small quantity of a trihydroxy-benzene sufficient substantially to retard discoloration of the product.

5. The method of stabilizing the characteristics of a low boiling normally light colored distillate petroleum product of the class of gasoline or kerosene that normally tends to become discolored during storage, which comprises adding thereto prior to substantial spontaneous discoloration a small quantity of pyrogallol sufficient substantially to retard spontaneous color formation.

6. The method of stabilizing the characteristics of a low boiling normally light colored distillate petroleum product of the class of gasoline or kerosene that normally tends to become discolored during storage, which comprises adding to the said product prior to any substantial self-generated discoloration a quantity of pyrogallol in the proportion of not more than 0.01% of pyrogallol but sufficient substantially to retard said discoloration.

7. A substantially water white color low boiling distillate petroleum fuel product which comprises a low boiling distillate petroleum product of the class of gasoline or kerosene which normally tends to become discolored upon storage having added thereto a small quantity of pyrogallol in amount sufficient substantially to retard the aforesaid discoloration and insufficient in amount to impart substantial color to the product.

JAMES B. RATHER.

ORLAND M. REIFF.

LESLIE C. BEARD, JR.

135